

## UNITED STATES PATENT OFFICE

2,188,214

## ROAD SURFACING

Carl Alexander Agthe, Zurich, Switzerland, assignor to J. R. Geigy A. G., Basel, Switzerland

No Drawing. Application December 14, 1938, Serial No. 245,770. In Switzerland December 23, 1937

2 Claims. (Cl. 106—32)

Road surfacing materials consisting of small stone and tar have the disadvantage of remaining soft after their laying on to the road, until the tar has thickened sufficiently by the partial evaporation of its oils and by oxidation and polymerisation. It usually takes several days until the tar coating has become hard and during this period the road surface suffers through indentation by vehicles passing over it.

10 Tar coatings of sufficient resistance can be obtained by the use of tars which are semi-solid to solid at atmospheric temperature. In this case however the tar made thinly fluid by heating must be mixed with hot stones and the mixed materials spread and rolled while in hot condition. After cooling a hard layer is obtained. This way of working which is often used for asphalt and bitumen layers, does not give good results with tar because a tar thickened up to a solid consistency 15 gives a brittle layer when admixed with stones. The insufficient adhesiveness of highly thickened tar is still further reduced when the tar has been heated to the high temperature necessary to enable the separate fragments of the stones to be 20 properly coated.

It has now been found that it is possible to produce tarred layers without the stated disadvantages if a mixture of small stone such as chippings or sand, it may be with additions such as 25 mineral fillers, cement and so forth, is first prepared with the usual fluid to viscous street tar, and a stiffening of the mass is then effected by means of an admixed pulverized condensation 30 product obtained by condensing with an aldehyde, preferably formaldehyde, a pine wood pitch of substantial insolubility in petroleum hydrocarbons, being the residue from the extraction of fine wood oil with a solvent, and described in the U. S. Patent 2,115,496. In this use the said 35 finely pulverized condensation product very easily dissolves in tar at atmospheric temperatures and surprisingly produces at such temperatures a considerable increase in the viscosity of the tar. The harmful effects of too high temperatures on 40 the tar are thus avoided. What is most extraordinary is that such condensation products exert their action even in very small proportions of less than 1% (calculated on the mixed material); they thus stand in a special position compared 45 with resins or pitches.

The working method of the invention affords particular advantages in the production of fine tar concrete which contains much fine mineral and mineral filler because the fine grain stone 50

is more easily coated by a fluid tar than by a pasty to solid binding agent.

According to the present process the usual street tar of thin fluid to thick fluid consistency can be used for coating the stone material. Tar bitumen mixture, oxidized tars such as so-called weather tar and tar with refining agents can also be used. If the thin fluid tar is chosen the coating of the stone can be effected in the cold but with the use of thickly fluid tar the mixture must be prepared hot. The pulverized condensation product is best added directly to the cold or hot mixture in the mixing chamber. If the hot process is used there is no danger of the tar suffering too high a temperature because such tars can 10 be chosen for the present process which by heating to temperatures below 120° C. are already so thinly fluid that they can easily be mixed with the stone. The pulverized condensation product can also be added subsequently to a prepared 15 mixture. It is only important that the powder should come into contact with fresh tar mixture and not with mixture which has been laid for some time. To achieve the desired effect care must also be taken that the powder used has as 20 fine and uniform a degree of sub-division as possible.

The pulverized condensation product can also be used mixed with inorganic or organic powders as for example mineral fillers, cement, ground 25 brown or hard coal and similar materials.

## Example 1

To 200 kg. of stone material consisting of equal parts of 3-6 mm. chippings, 1-3 mm. chippings and 0-3 mm. broken sand are added 8 kg. of lime powder and then while warming the stone to about 50-60° C., 15 kg. of street tar having a viscosity of 40 sec. measured in the tar consistency meter at 30° C., which have been heated 35 to 70-80° C. are admixed. 0.6 kg. of finely pulverized condensation product of the aforesaid nature is then strewn on to the still warm mixture in the mixing chamber while stirring.

## Example 2

To 200 kg. of stone consisting of two parts by volume of 3-6 mm. chippings and three parts by volume of 0-3 mm. broken sand, after the addition of 13 kg. of lime powder, 20 kg. of a thin fluid tar having a viscosity of about 3 sec. measured at about 30° C., are added when heating and then while stirring 2 kg. of a mixture of two parts of pulverized condensation product of the 50 55

aforesaid nature and three parts of lime powder are strewn on.

*Example 3*

- 5 To 200 kg. of stone consisting of two parts by volume of 5-8 mm. chippings, 2½ parts by volume of 0-3 mm. broken sand and half part by volume of pit sand, 10 kg. of mineral filler are added and thereupon 14 kg. of street tar having a viscosity of 200-300 sec. measured at 30° C. are stirred into 10 a homogeneous mixture, the stone material being heated to 60-80° C. and the tar to about 100° C. To this is added 0.8 kg. of a mixture of two parts of the aforesaid pulverized condensation product and three parts of ground brown coal. The mixture must be worked in hot condition because after cooling it forms an extremely hard mass.

The process according to the invention may also be performed in such a way that a layer from stones or sand is impregnated with a fluid tar 20 and then intermixed by means of hoe- or plough-like implements with the aforesaid powdered condensation product. Inversely it is also possible to first incorporate to the stone or sand layer the aforesaid powdered condensation product and to thereupon add the fluid tar thereto.

It is already known to produce macadam layers by coating broken stone first with a fluid or

semi-fluid binding agent and then with a resin or pitch in dust or powder form. In contradistinction the condensation product used according to the invention does not serve as a binding agent as is apparent from the very small quantity used of less than 1%. In Example 3 the quantity of the aforesaid condensation product amounts to but 0.14% calculated on the mixture. In the present process only the fluid to thick fluid tar which is added direct to the stone material, acts as a binder. The sole function of the aforesaid condensation product is to stiffen the mixture.

What I claim is:

1. A process for stiffening road making layers 15 of small stone and tar, characterized in that a pulverized condensation product obtained by condensing with an aldehyde a pine wood pitch of substantial insolubility in petroleum hydrocarbons, being the residue from the extraction of 20 pine wood oil with a solvent, is added to the road making mixture before or during its laying.

2. A process according to claim 1, characterized in that the aforesaid pulverized condensation product is used mixed with organic or inorganic powders.

CARL ALEXANDER AGTHE.